

## UNITED STATES PATENT OFFICE

2,137,144

## PROCESS FOR THE PRODUCTION OF METAL CARBIDES

Nicolas Sanderichin, Paris, France, assignor to  
Follsain Syndicate Limited, London, EnglandNo Drawing. Application October 23, 1937, Serial  
No. 170,703. In Great Britain January 9,  
1936

3 Claims. (Cl. 23—208)

This invention relates to the production of carbides of metals such as iron, tungsten, titanium, chromium, and molybdenum but is not concerned merely with the formation of a surface zone of carbides on such metals.

5 The object of the present invention is to devise an improved process for the formation of such carbides by which good quality carbides will be obtained and the invention consists in a process 10 for the production of metal carbides which consists in heating the metal (of which the carbide is to be formed) in a finely divided condition in admixture with a carburizing mixture containing manganese dioxide, in a hermetically sealed 15 box.

Further features of the invention will be apparent from the description given hereafter.

In carrying my invention into effect in one convenient manner I form my improved carburizing 20 material for the formation of metal carbides from a mixture of finely divided charcoal or other suitable form of carbon, caustic potash, manganese dioxide and ammonium chloride and while the proportions in which the various ingredients 25 are mixed together may be varied to suit any particular requirements, I find the following mixture to be suitable, namely,

|                         | Kilograms  |
|-------------------------|------------|
| Finely divided charcoal | 1.         |
| Caustic potash          | 0.15       |
| Manganese dioxide       | 0.1 to 0.3 |
| Ammonium chloride       | 0.05       |

The metal to be treated, for example, in the form of ferro tungsten or tungsten metal, ferro 35 titanium or titanium metal, ferro molybdenum or molybdenum metal, or the like is finely divided as by grinding and mixed with the carburizing mixture and packed in a hermetically sealed box in such a manner to avoid so far as possible the 40 occlusion of air but in actual operation under heat the ammonium chloride will expel the occluded air from the mixture.

The sealed box is heated in a furnace to a temperature of 1200° C. for about 1½ to 2 hours 45 and the metal carbide obtained by the process after cooling slowly while protected from the air, may be utilized for any desired purpose. For

example, when producing an alloy in which high hardness and great toughness are required I may use a mixture resulting in a product having the following proportions:—

| Percent             | 5  |
|---------------------|----|
| Carbide of iron     | 30 |
| Carbide of tungsten | 70 |

For a tool steel I should use a mixture consisting of:—

| Percent             | 10 |
|---------------------|----|
| Carbide of iron     | 20 |
| Carbide of tungsten | 70 |
| Carbide of chromium | 10 |

For dies, the ingredients and proportions would be:—

| Percent             | 15 |
|---------------------|----|
| Carbide of iron     | 75 |
| Carbide of chromium | 25 |

The carbides produced by my process contain 20 no manganese, or if manganese be present, it is in so small a quantity as not to affect the properties of the carbide.

I may vary the constituents in my improved mixture and the proportions in which they are 25 incorporated and the temperature at which the carburizing process is carried out depending upon the nature of the metal to be treated or any practical requirements which may have to be fulfilled.

I claim:

1. The process for the production of metal carbides which consists in heating at least one metal selected from the group consisting of iron, tungsten, titanium, chromium, and molybdenum in a 35 finely divided condition in admixture with a carburizing mixture consisting of charcoal, manganese dioxide, caustic potash and ammonium chloride.

2. A process as claimed in claim 1 wherein the 40 carburizing mixture consists of 100 parts charcoal, 10 to 30 parts manganese dioxide, 15 parts caustic potash and 5 parts ammonium chloride.

3. The process as claimed in claim 1 wherein 45 the heating step is carried out at a temperature of 1200° C.

NICOLAS SAINERICHIN.